

**3,519,418**  
**AGE-HARDEENABLE NICKEL-BASE**  
**BRAZING ALLOY**

Paul R. Mobley and Reed E. Yount, Cincinnati, Ohio,  
 assignors to the United States of America as represented by the Secretary of the Air Force  
 No Drawing. Filed Apr. 22, 1968, Ser. No. 723,232  
 Int. Cl. C22c 19/00

U.S. Cl. 75—170

5 Claims

### ABSTRACT OF THE DISCLOSURE

Age-hardenable nickel-base brazing alloys are provided which possess strength and oxidation resistance in the 1700° F. to 1900° F. temperature range. The alloys contain as essential ingredients 3 to 10 percent silicon, 2 to 4 percent titanium, 1 to 3 percent aluminum, 1 to 20 percent of at least one of the alloying elements selected from the group consisting of chromium, cobalt, boron and iron, and the balance being nickel accompanied by unavoidable impurities.

### BACKGROUND OF THE INVENTION

The present invention relates to age-hardenable nickel-base brazing alloys and, more particularly, to nickel-base alloys having a particularly high combination of strength properties and oxidation resistance in the temperature range of from about 1700° F. to approximately 1900° F.

It is well known that there are a number of age-hardenable nickel-base alloys available to the art for use at room temperature as well as at elevated temperatures. These prior art alloys, however, possess certain disadvantages either from the standpoint of strength or from the standpoint of oxidation resistance. In addition, many of the

TABLE I.—ALLOY CONSTITUENTS IN PERCENT BY WEIGHT

| Alloy No. | Ni   | Cr    | Co    | Si   | Fe    | B   | Ti  | Al  | Brazing temp., ° F. |
|-----------|------|-------|-------|------|-------|-----|-----|-----|---------------------|
| 1.....    | 68.0 | 7.0   | ..... | 5.0  | 2.0   | 2.9 | 3.0 | 2.0 | 2,050               |
| 2.....    | 89.6 | ..... | ..... | 3.5  | ..... | 1.9 | 3.0 | 2.0 | 2,050               |
| 3.....    | 70.2 | ..... | 18.0  | 4.5  | ..... | 3.3 | 3.0 | 2.0 | 2,050               |
| 4.....    | 69.0 | 17.0  | ..... | 10.0 | ..... | 3.0 | 3.0 | 2.0 | 2,050-2,150         |

prior art nickel-base alloys, although possessing satisfactory strength properties, are characterized by an unsatisfactorily low oxidation resistance, especially at elevated temperature.

Designers of equipment for use at high stress and elevated temperatures require that nickel-base alloys possess a yield strength representing a high proportion of the tensile strength thereof since the yield strength is the property of the alloy employed by the designer. Also, age-hardenable nickel-base alloys having improved oxidation resistance in combination with improved strength properties are required by the art for use at elevated temperatures. Although attempts have been made to overcome the aforementioned difficulties, none have been entirely successful when carried into practice on a commercial basis. In further attempts to overcome the difficulties of the prior art, however, it has been discovered that age-hardenable nickel-base alloys containing specially controlled and coordinated amounts of alloying elements possess an improved and outstanding combination of high strength and oxidation resistance in the temperature range from about 1700° F. to about 1900° F.

### SUMMARY OF THE INVENTION

In accordance with this invention novel age-hardenable nickel-base alloys are formulated from an admixture of specially controlled amounts of certain alloying ingredients. The combination of ingredients provide the alloys

with the necessary elevated temperature strength and oxidation resistance needed for use in the fabrication of structural components subjected to the stress and strain of high temperature operational conditions. The alloys contain nickel, silicon, titanium and aluminum as essential ingredients, together with one or more alloying ingredients selected from the group consisting of chromium, cobalt, boron and iron.

Accordingly, it is the primary object of the present invention to provide age-hardenable nickel-base brazing alloys having improved combinations of high strength and high oxidation resistance at elevated temperatures.

Another object of the present invention is to provide improved nickel-base alloys of specially controlled compositions which exhibit high strength and oxidation resistance at elevated temperatures in the range of 1700° F. to 1900° F.

Other objects and advantages of the invention will become apparent from the following detailed description thereof.

### DESCRIPTION OF THE PREFERRED EMBODIMENT

Pursuant to the above objects, the present invention 25 contemplates a nickel-base brazing alloy containing about 3% to about 10% silicon, about 2% to 4% titanium, about 1% to about 3% aluminum, 1% to 20% of at least one of the alloying ingredients selected from the group consisting of chromium, cobalt, boron and iron, and the 30 balance essentially nickel accompanied by unavoidable impurities. These alloys are characterized by a very high combination of strength and oxidation resistance at temperatures from about 1700° F. to 1900° F.

Typical alloys prepared in accordance with the invention 35 are presented in Table I, while Table II presents hardness data for the alloys described in Table I.

TABLE II.—HARDNESS DATA (Rc)

| Alloy No. | As-brazed | Aged                |                     |                    |
|-----------|-----------|---------------------|---------------------|--------------------|
|           |           | 1,200 ° F., 24 hrs. | 1,400 ° F., 16 hrs. | 1,650 ° F., 4 hrs. |
| 1.....    | 52.0      | 51.5                | 52.5                | 62.0               |
|           | 50.8      | 50.5                | 50.8                | 45.0               |
|           | 50.0      | 50.5                | 50.8                | 51.3               |
|           | 53.5      | 50.5                | 49.5                | 48.7               |
|           | 53.5      | .....               | .....               | .....              |
| 2.....    | 59.0      | 56.5                | 58.0                | 56.5               |
|           | 57.5      | 57.0                | 54.5                | 54.0               |
|           | 58.5      | 57.0                | 58.0                | 56.0               |
|           | 57.5      | 56.0                | 57.0                | 54.0               |
|           | 58.5      | 58.5                | 59.5                | .....              |
| 3.....    | 59.5      | 56.5                | 56.0                | 56.0               |
|           | 55.0      | 54.5                | 58.5                | 55.5               |
|           | 52.5      | 54.5                | 53.0                | 53.4               |
|           | 55.0      | 55.0                | 56.0                | 54.8               |
|           | 55.0      | 58.5                | 57.0                | 54.3               |
| 4.....    | 56.0      | 53.5                | 57.5                | 54.8               |
|           | 56.0      | 57.5                | 57.5                | 56.0               |
|           | 57.5      | 58.0                | 59.5                | 57.5               |
|           | 57.5      | .....               | .....               | .....              |
|           | 58.0      | .....               | .....               | 54.3               |

The alloys may be prepared by conventional techniques such as non-consumable electrode melting under a partial argon atmosphere with the heat source a TIG welding torch oscillated over the charge. The alloys may also be produced by other conventional methods where a controlled atmosphere is used. For example, in preparing a desired brazing alloy, the ingredients are charged, in weighed increments, into an arc melting furnace which may comprise a water-cooled copper crucible and a tung-

sten electrode. The charge is melted under an inert atmosphere such as argon or helium to prevent contamination of the melt. The resulting melt is then solidified into an ingot. These alloys can be comminuted into small chunks or to a powder as desired. In its powder condition, the alloys can be uniformly mixed with a binder such as nitrocellulose or an acrylic resin to form a paste, it being essential that the binder burn away leaving no ash to contaminate the brazed joint.

In whatever form prepared, the braze material is placed about the surfaces to be joined. The furnace used should be capable of reaching a temperature of about 2500° F. For example, the joint and surrounding braze material may be heated by a radio frequency induction heater to above the liquidus of the brazing alloy and held at temperature until the melted alloy is observed to melt and flow freely over the surfaces to be joined. At this point the heating means is switched off and the melted alloy allowed to freeze to form the brazed joint.

Brazed T joints have been made successfully in accordance with this procedure and with the alloys within the scope of the invention. All were brazed at approximately 2050° C.

Unless otherwise indicated, the term percent, as used in the instant specification and appended claims, refers to 25 percent by weight based on the total alloy weight.

Although the present invention has been described with reference to preferred embodiments, those skilled in the art will readily understand that various modifications and alterations may be resorted to without departing from the spirit of the invention and that all such modifications as fall within the scope of the appended claims are intended to be included therein.

We claim:

1. A nickel-base brazing alloy consisting essentially 35 75—171; 148—32.5, 162 of about 3 to 10 percent silicon, 2 to 4 percent titanium,

1 to 3 percent aluminum, 1 to 20 percent of at least one of the alloying elements selected from the group consisting of chromium, cobalt, boron and iron; and the balance being nickel accompanied by unavoidable impurities.

5 2. A nickel-base brazing alloy in accordance with claim 1 consisting essentially of about 5 percent silicon, 3 percent titanium, 2 percent aluminum, 7 percent chromium, 2 percent iron, 2.9 percent boron, and the balance being nickel accompanied by unavoidable impurities.

10 3. A nickel-base brazing alloy in accordance with claim 1 consisting essentially of about 3.5 percent silicon, 3 percent titanium, 2 percent aluminum, 1.9 percent boron and the balance being nickel accompanied by unavoidable impurities.

15 4. A nickel-base brazing alloy in accordance with claim 1 consisting essentially of about 4.5 percent silicon, 3 percent titanium, 2 percent aluminum, 3.3 percent boron, 18 percent cobalt and the balance being nickel accompanied by unavoidable impurities.

5 5. A nickel-base brazing alloy in accordance with claim 1 consisting essentially of about 10 percent silicon, 3 percent titanium, 2 percent aluminum, 17 percent chromium and the balance being nickel accompanied by unavoidable impurities.

#### References Cited

#### UNITED STATES PATENTS

|           |        |             |        |
|-----------|--------|-------------|--------|
| 2,875,043 | 2/1959 | Tour        | 75—171 |
| 2,899,302 | 8/1959 | Cape et al. | 75—170 |

RICHARD O. DEAN, Primary Examiner

U.S. Cl. X.R.